

Aug. 30, 1960

B. G. FIRTH

2,950,994

METHOD FOR PREPARING COLD CATHODES AND RESULTING ARTICLE

Filed Feb. 25, 1959



INVENTOR  
*BERNARD G. FIRTH*  
BY  
*Eyre, Mann & Lucas*  
ATTORNEYS

# United States Patent Office

2,950,994

Patented Aug. 30, 1960

1

2,950,994

## METHOD FOR PREPARING COLD CATHODES AND RESULTING ARTICLE

Bernard G. Firth, Newark, N.J., assignor to Tung-Sol  
Electric Inc., a corporation of Delaware

Filed Feb. 25, 1959, Ser. No. 795,514

9 Claims. (Cl. 117—222)

The present invention relates to electric discharge devices of the type wherein the current carriers are electrons emitted from a coated electrode and comprises a coating for such type electrode which has improved electron emissive characteristics. The invention includes also a method of preparing and applying a coating composition to the metal of the electrode which is commercially practicable and insures optimum physical condition of the applied coating. The invention will be described with reference to a cathode coating for a cold cathode vacuum tube of the type disclosed in the copending joint application of the present applicant and Albert M. Skellet, Serial No. 697,928, filed November 21, 1957, and entitled "Starting Means for Cold Electrode Vacuum Tube Devices."

It has heretofore been known that a magnesium oxide coating, when so prepared as to be porous and formed of microscopic needle-like or stalactite-like structures, will give off a copious and self-sustaining stream of electrons when bombarded with primary electrons. (See Dobischek et al. Patent No. 2,802,127.) No commercially practical method of forming such coating has heretofore been known nor have cold cathode vacuum tubes been produced heretofore which could carry relatively high currents. For example, about 30 milliamperes per square centimeter of coating is about the maximum current obtainable from magnesium oxide coatings of the prior art. In accordance with the present invention cold cathodes have been prepared that are capable of sustaining currents of the order of 145 milliamperes per square centimeter.

In accordance with the invention a mixture of magnesium oxide, basic magnesium carbonate powder and a thinner is first prepared. The mixture is then milled in a ball mill jar with pebbles of selected graded size for an extended period of time and at a predetermined rate of rotation. After milling additional thinner is added and the so prepared coating is sprayed on the electrode while the electrode is rotated at a predetermined relatively high rate. Each of the above described steps of the new process contributes to the improvement in the quantity of electron emission from the coated electrode.

The single figure of the accompanying drawing is a perspective view, partly broken away, of a cold cathode tube having a coated cathode therein prepared in accordance with the invention.

The cold cathode vacuum tube illustrated in the drawing comprises an outer glass envelope 2 sealed to a button type glass base 4. A cylindrical cathode 6 prepared in accordance with the invention is mounted on the base 4 by means of a conductive support which is fused through the base and connected to a pin terminal 8. The cathode 6 comprises a cylindrical oxidized nickel sleeve 10 upon the exterior surface of which is the electron emissive coating 12. Also within the evacuated envelope 2 and mounted on the base 4 are a collector

2

electrode 14, a metal shield 16 and a starter electrode 18. Electrodes 14 and 18 are connected respectively, through suitable conductive supports to pin terminals 20 and 22. Collector electrode 14 is of mesh construction. Starter electrode 18 comprises a wire of tungsten having a fine pointed tip directed toward coating 12 of the cathode, an opening of the collector electrode being aligned with the starter electrode for unobstructed passage to the coating of primary electrons given off by field emission from the starter tip when a high negative potential with respect to the cathode is impressed upon the starting electrode.

To prepare the coating 12, and assuming the cathode sleeve to be of about  $5\frac{1}{16}$ " outer diameter, a mixture of 15 paste-like consistency is first obtained by combining

Magnesium oxide, reagent grade \_\_\_\_\_ grams 24  
Basic magnesium carbonate U.S.P. heavy powder  
( $MgCO_3$ )<sub>4</sub>  $Mg(OH_2)$ . $nH_2O$  \_\_\_\_\_ grams 24  
20 Amyl acetate, purified (thinner) \_\_\_\_\_ cc 300

The paste-like composition is then milled in a one quart porcelain ball mill jar one-half full of selected flint pebbles of  $\frac{3}{8}$ " to  $\frac{5}{8}$ " size, the charge just covering the pebbles. The ball mill jar is rotated at a speed of 25 90 r.p.m. for 20 hours following which additional amyl acetate, about 420 cc., is added. The milling reduces the particle size to approximately 0.5 to 2.0 microns. Milling for longer than 20 hours does not appreciably 30 reduce particle size. Milling for a shorter period of time, for example, 5 hours, gives a wider range of particle size say from 1 to 10 microns. If the coating mixture is fully thinned prior to milling the relatively uniform and small particle size is not obtained.

To apply the composition to the cathode sleeve, the 35 sleeve is rotated at 150 r.p.m. while sprayed with the milled composition using a spray type gun under an air pressure of 20 lbs. Spraying is continued until the coating thickness is from 28 to 48 microns and the coating weight from 1.4 to 1.6 milligrams per square centimeter.

With a cathode coating of the above described initial 40 composition prepared and applied as above described, copious and self-sustained emission of electrons results once the emission is initiated either by a stream of primary electrons, as from the point of the starter electrode 45 of the device, or by a spark coil or as a result of illumination by ultraviolet light. When a collector electrode such as electrode 14 is maintained positive with respect to the cathode by application of a suitable voltage thereto 50 conduction through the tube will be maintained. It is believed that the high rate of electron emission and the self-sustaining feature thereof is due to the porous or spongy character of the coating when prepared as above 55 described. A radial potential gradient appears to be set up in the coating which causes "avalanche" emission of electrons. The addition of basic magnesium carbonate to the magnesium oxide, the fine particle size obtained by milling prior to final thinning and the high rate of travel of the surface to be coated transverse to the direction 60 of the spray are each important to the preparation of a coating of excellent electron emission characteristics.

The invention has now been described with reference to the preparation of a cold cathode for vacuum tubes. Obviously the new coated electrode of the invention could 65 be of other than cylindrical shape and could be advantageously employed in tubes other than the diode illustrated in the drawing. Various changes in the detailed process described could be made without departing from the spirit of the invention or the scope of the accompanying 70 claims. For example, although amyl acetate has been given as the thinner, any thinner could be used that does not leave a harmful deposit, such as carbon, on the

coating and that dries at a suitable rate for the practice of the spray coating process. Various other proportions of the constituents of the coating could be employed. Although the cathode sleeve rotation during spray coating was given as 150 r.p.m. higher rates could be used if desired.

The following is claimed:

1. An electrode for vacuum tubes comprising a metal base having a porous, spongy coating thereon derived from a paste comprising a thinner and fine particles of magnesium oxide and basic magnesium carbonate, said coating having a high electron emission rate.

2. The electrode according to claim 1 wherein said coating is from 28 to 48 microns thick and of a weight per square centimeter of area of 1.4 to 1.6 milligrams.

3. The electrode according to claim 1 wherein said paste comprises substantially equal parts by weight of magnesium oxide and basic magnesium carbonate.

4. The electrode according to claim 1 wherein the particle size of said coating is from 1 to 2 microns.

5. The method of preparing a coating having high electron emission rate for metal electrodes for vacuum tubes comprising preparing a paste of magnesium oxide, basic magnesium carbonate and a thinner, milling the paste to reduce particle size to about 1 micron, thinning the milled paste and finally spraying the metal surface

of the electrode with the thinned paste while rotating the electrode at a rapid rate.

6. The method of preparing a coating having a high electron emission rate for a metal electrode which comprises preparing a paste of magnesium oxide, basic magnesium carbonate and a thinner, milling the prepared paste to reduce particle size to at least about 2 microns, thinning the milled paste and finally spraying the outer surface of the metal electrode with the thinned milled paste while rapidly rotating the electrode.

7. The method according to claim 6 wherein the metal electrode is rotated at about 150 revolutions per minute.

8. The method according to claim 6 wherein the paste is prepared from substantially equal parts by weight of magnesium oxide and basic magnesium carbonate and wherein the thinner is amyl acetate.

9. The method according to claim 6 wherein milling of the paste is effected in ball mill jars with flint pebbles of  $\frac{3}{8}$ " to  $\frac{7}{8}$ " size at a rate of rotation of about 90 r.p.m. for about 20 hours.

References Cited in the file of this patent

UNITED STATES PATENTS

|    |           |                        |               |
|----|-----------|------------------------|---------------|
| 25 | 1,874,785 | Miller et al. -----    | Aug. 30, 1932 |
|    | 2,433,821 | Toorks -----           | Dec. 30, 1947 |
|    | 2,873,218 | Dobischek et al. ----- | Feb. 10, 1959 |